

Patented Apr. 12, 1927.

1,624,492

# UNITED STATES PATENT OFFICE.

ARTHUR D. LITTLE, OF BROOKLINE, AND CARROLL E. CARPENTER, OF MELROSE, MASSACHUSETTS, ASSIGNORS TO ARTHUR D. LITTLE, INC., OF BOSTON, MASSACHUSETTS, A CORPORATION OF MASSACHUSETTS.

## PAPER MANUFACTURE.

No Drawing.

Application filed March 30, 1925. Serial No. 19,283.

Our present invention relates to the art of making paper from wood pulp, and particularly to the manufacture of newsprint paper. Its object is to make available for the uses of that manufacture, and for analogous uses, certain woods, particularly the southern pines of various species and southern hard woods of the class known as gumwood, which have heretofore been found unsuitable for those purposes, although readily obtainable in large quantities and at relatively low prices.

Our invention comprises the preparation of a fiber furnish of chemical pulp from southern pine and a major component of mechanical pulp of southern gumwood, with such treatment of the gumwood or the furnish as will cause the furnish to be sufficiently feltable so that it will pass over the paper making machine. Our invention more particularly includes the transforming of an unworkable wood fiber mixture or furnish composed of the aforesaid ingredients into a furnish that is workable on the paper machine, by the incorporation in the unworkable furnish of a flocculent agglutinant, preferably colloidal cellulose, conveniently, but not necessarily, produced by hydrating a part of one of the ingredients of the unworkable furnish. Our invention also embraces the method or steps involved in so transforming such a furnish, and the resulting products, including the finished product, newsprint paper made from southern pine and gumwood; as will more fully appear from the following detailed description.

Preliminary to a description of the invention, a brief discussion of the qualities required in newsprint paper, and of the characteristics, with reference to the making of paper, of the woods above named and those heretofore used for making newsprint paper, will be helpful. Newsprint paper must have strength enough to carry it through the printing press at high speed, proper body and hardness, and an absorptive quality sufficient to absorb quickly the liquid vehicle of the newspaper printing inks. It must also be light in color, as nearly white as practicable. These conditions have been met heretofore by making such paper of a mixture of chemical wood pulp, the relatively long fibers of which give the required tensile strength, and ground wood pulp to give the

required body and absorptive qualities and 55 reduce the cost. Substantially the entire commercial output of such paper is now, and long has been, made from the woods of the northern conifers, namely, spruce, fir, hemlock, larch, etc.; chemical pulp being made 60 from these woods by the sulphite process. The ground wood pulp always predominates largely over the chemical pulp, and a very common proportion is seventy-five percent of the former to twenty-five percent of the 65 latter.

The southern pine woods have fibers much longer than those of the northern conifers, but they also have a high content of resin, many times that of the northern conifers. 70 On account of this high resin content, the southern pines cannot be advantageously made into pulp by the sulphite process or by grinding. A long fibered stock may be readily prepared from the southern pines by 75 the sulphite process, but the pulp so made, known as kraft pulp is brown in color and therefore is not suitable, without at least partial bleaching, as a component in newsprint and other white papers. 80

The gumwoods are white in color, and have relatively short fibers and a low resin content, wherefore they are well adapted to be made into pulp by grinding and the mechanical pulp so made from gumwood has 85 the color and absorptive qualities required of the ground wood component of newsprint paper.

But when mechanical pulp is produced from gumwood by methods of grinding at 90 present ordinarily practiced, the separate particles of the wood thus obtained are so short in average length, and have such inferior felting qualities, that such pulp cannot be handled by the paper machine and 95 made into satisfactory newsprint paper either alone or in admixture with permissible proportions of long fibered chemical pulp.

For the reasons above indicated no newsprint paper is now made in the South or 100 from southern woods, notwithstanding that the consumption of such paper in the Southern States is in the neighborhood of fifteen hundred tons per day, and that vast quantities of gumwoods and southern pines are 105 found in the Southern States in convenient access to the markets in those States; and in spite of the fact, also, that the prices of

these woods have for many years been much lower than the prices of pulp wood in the North.

The primary problem involved in attaining our object of making available to the paper industry, for the purposes above stated, the great supplies of southern pines and gumwoods, was to find a means by which gumwood ground pulp, in admixture with permissible proportions of long-fibered chemical pulp, could be made into a workable paper furnish. In the search for a solution of this problem we have carried out a long and costly series of experiments, in the course of which we have attempted to obtain, by grinding gumwood with a wood pulp grinder of the type now commercially used, mechanical pulp which, in admixture with permissible proportions of long-fibered chemical pulp would pass over the paper machine. Although we made many such attempts, with various adjustments of the wood pulp grinder and with various modifications in the dressing of the stones, the fibers of the wood were so generally broken into short lengths by the grinder, that we were not able to obtain from gumwood by such means, mechanical pulp of the felting qualities and other characteristics required of the ground wood component of newsprint paper.

We succeeded, and were the first to succeed, in bleaching southern pine sulphate pulp, by careful control of the bleaching process, to a color which permits of its use in white paper, with conservation at the same time of the necessary strength of the fibers, thus solving the secondary problem of making this pulp usable as the long-fibered feltable component of such paper. But paper made entirely of such bleached sulphate fiber or with a major component thereof in admixture with gumwood ground pulp, is not suitable for newsprint paper, while fiber mixtures containing permissible proportions of such sulphate pulp and the quality of gumwood pulp which we were able to obtain by grinding, are unworkable.

The primary problem was solved by our discovery that the addition of a small proportional content of a suitable flocculent agglutinant to the furnish or pulp mixture of sulphate fiber and mechanical gumwood pulp, so changed the working properties of the furnish that a web of good formation was readily secured which would run well over the paper machine, presented no unusual difficulties in manufacture and made finished paper possessing the requisite strength and printing qualities for use on high speed newspaper printing presses. The proportion of agglutinant which we have found suitable is from five to ten percent by weight of the dry fiber contained

in the total furnish; although a somewhat larger or smaller proportion may be used within the protection of our claims.

The agglutinant material causes the otherwise unfeatable fibers to mat and interlock into a firm web, and to adhere together. It also retards the draining away of water from the pulp on the wire of the paper machine, so that more time is given for the fibers to thus interlock and felt together, before the water is drawn out by the suction boxes at the delivery end of the wire.

The water which is pulled out by the suction boxes carries with it part of the agglutinant, to wit, all that does not remain adhering to and in mesh with the fibers lying on the wire. This water is used, in part at least, over and over again, being continuously returned to the stuff chest of the paper machine, and there added to the stock which is delivered from the beater. Hence the water is a carrier or vehicle for the agglutinant, and continually supplies the agglutinant to the paper stock in the machine. Whatever the exact action of the agglutinant may be, its effect is a treatment of the gumwood to make the fibers thereof feltable with one another and with the long fibers of the pine pulp, into a firm and strong web. It transforms an otherwise unworkable pulp mixture into a furnish which can be satisfactorily handled by a paper machine and made thereby into suitable newsprint paper. After extraction of the water, enough of the agglutinant remains in the web to serve as a binder adhering to the fibers and cementing them together, thus making the finished paper hard and strong enough to meet the requirements of commercial newsprint paper.

The agglutinant preferably used is colloidal cellulose made by beating chemical wood pulp, or otherwise abrading it in water, until it is hydrated to the colloidal state. Cellulose so prepared is flocculent in condition, and is pure cellulose, free from any compounds or ingredients liable to produce objectionable results in the paper. It may be made from any chemically prepared or cooked wood fiber, including chemical pulp of southern pine or southern gumwood, or from other suitable cellulose material, but preferably is made from the same bleached sulphate fiber as is used in the pulp furnish. Proper transformation of wood fiber to the colloidal state may be effected by beating in a standard beater, for a period of from twelve to fifteen hours; but it may be more quickly effected, in about three hours, by treatment continuously and in rotation by a beater and a Jordan engine connected in series.

As more particularly illustrating the nature and characteristics of our invention, we give as follows a description of the

exact procedure and ingredients which were used in making a certain run of paper according to the invention, without however implying any limitation of our protection to the exact steps, ingredients, or proportions so described. The furnish was composed of:

|                                      | Per cent. |
|--------------------------------------|-----------|
| No. 1 quality southern pine sulphate |           |
| 10 pulp, bleached                    | 20        |
| Ground black gumwood                 | 70        |
| Colloidal cellulose                  | 10        |

To the above total fiber furnish there was added, for the usual purpose of sizing, 15 1½% of rosin size and 1% of alum. The sulphate pulp was made from North Carolina pine and was bleached by standard chlorine bleaching equipment. The ground pulp was made from black gumwood obtained from the swamps of the Pearl River, 20 Mississippi; by the operation of a standard wood pulp grinder with a stone commonly used for the production of pulp for newsprint use. The stone was of medium grit buried with a four-cut straight burr and operated with a grinding pressure of thirty pounds per square inch on a fourteen inch cylinder. The colloidal cellulose was made from chemical wood pulp by hydration in 25 a standard beater and Jordan, connected in a series and operated in repeated rotation on the stock. The furnish thus constituted was made into paper on a standard Fourdrinier paper machine, which was run in 30 the usual way for making newsprint paper.

Paper made as thus particularly described has been used with entire satisfaction in printing the regular editions of 35 daily newspapers on high speed rotary perfecting newspaper presses of types which make exacting demands on the paper web.

While the specific proportions of the ingredients illustratively described above are preferred at present to others, nevertheless 40 considerable variations in such proportions may be made, and equivalent ingredients may be substituted, within the protection herein claimed. For instance, the southern pine sulphate fiber and gumwood fibers may be used in other proportions, although 45 always with a substantial preponderance of the ground fiber; and other flocculent agglutinants having the functions hereinbefore ascribed to the agglutinant may be 50 used in place of colloidal cellulose; while colloidal cellulose otherwise made in any 55 suitable manner may be used.

Our invention has thus made possible the manufacture of commercial newsprint paper 60 from southern pine and southern gumwood and has thereby rendered available to the industry great quantities of wood heretofore unavailable for this use.

While we have made this result possible 65 by modifying the fiber furnish, consisting

chiefly of mechanical gumwood pulp, by adding thereto an ingredient or agent, namely colloidal cellulose, which has the capacity of making an otherwise unworkable fiber mixture feltable into strong paper in a paper machine, nevertheless the protection which we claim is not limited to the use of an added felting agent or to paper containing such felting agent. Since we are the first to have produced a workable furnish composed wholly of southern pine chemical pulp and gumwood mechanical pulp, and are the first to make merchantable newsprint paper of these ingredients, we claim protection generically for 80 means and methods of making such workable furnish, and for our products, commensurate with the novelty of our invention:

The woods designated by the words "southern pine" as used in this specification include the following: short leaf yellow (*Pinus echinata*), long leaf yellow, and Georgia long leaf (*Pinus palustris*), Cuban pine (*Pinus heterophylla*), loblolly pine 85 (*Pinus serotina* or *Pinus taeda*), and, in general, all pines found in the southern United States and characterized by a resin content substantially greater than that of the northern conifers. The term "gumwood" as here used, includes black gum (*Nyssa sylvatica*), cotton gum (*Nyssa aquatica*), sweet or red gum (*Liquidambar styraciflua*), and the like.

What we claim and desire to secure by 100 Letters Patent is:

1. The method of making newsprint paper from a fiber furnish consisting of southern gumwood ground pulp and southern pine sulphate pulp, which consists in modifying 105 said furnish by incorporating colloidal cellulose therewith, in substantially the proportions specified, and then forming said modified furnish into a paper web.

2. The method of making newsprint paper which embraces supplying to the paper machine a fiber furnish having as one component a chemical pulp, as another and major component southern gumwood pulp of such character that it would not so felt with the chemical component that the furnish could be carried over the paper machine, and a flocculent agglutinant to modify the felting capacity of the furnish to enable it to be carried over the paper machine.

3. The method of making newsprint paper which embraces supplying to the paper making machine a furnish consisting of southern pine sulphate pulp, southern gumwood ground pulp; and material to effect a felting action between the two components, and forming said furnish into a paper web on the machine.

4. The method of making newsprint paper from southern pine and ground gumwood 130

5 pulp which consists in combining 70% to 80% ground gumwood and 30% to 20% southern pine sulphate pulp to provide a sufficiently felting furnish to pass over the paper making machine, and forming the furnish into a paper web.

6 5. The method of making newsprint paper from southern pine and gumwood which comprises preparing a fiber furnish of southern pine sulphate pulp and mechanically disintegrated gumwood, with treatment of the gumwood to make its fibers sufficiently feltable to enable the furnish to pass over the paper making machine, and forming said furnish into a paper web.

10 6. The method of making a paper furnish from southern pine sulphate pulp and gumwood ground pulp which consists in incorporating with said gumwood pulp chemical wood fiber colloidal cellulose in substantially the proportions specified.

15 7. The method of transforming an unworkable paper furnish consisting chiefly of mechanical gumwood pulp of such character that it would not be carried over the paper machine which comprises incorporating colloidal cellulose in said furnish in substantially the proportions specified and thereby causing the fibers to become feltable into a suitable paper web.

20 8. The method of making a newsprint pa-

per furnish from southern pine sulphate pulp and gumwood ground pulp which consists in combining said ingredients in the ratio of approximately 70% to 80% of the ground gumwood and the balance of southern pine sulphate pulp.

25 9. Newsprint paper composed of southern pine sulphate pulp, mechanical gumwood pulp, and colloidal cellulose.

10 40 10. Newsprint paper composed of a mixture of southern pine sulphate pulp, mechanical gumwood pulp, and a flocculent agglutinant.

11. A paper furnish for the manufacture 45 of newsprint paper consisting of southern pine sulphate pulp, southern gumwood ground pulp, and chemical wood fiber colloidal cellulose in substantially the proportions specified.

12. A paper furnish for the manufacture of newsprint paper consisting of southern pine sulphate pulp and gumwood ground pulp, and a felting agent in sufficient measure to make said furnish sufficiently feltable 55 to enable the furnish to pass over the paper making machine.

In testimony whereof we have affixed our signatures.

ARTHUR D. LITTLE.  
CARROLL E. CARPENTER.